

July 19, 1960

B. H. CARROLL ET AL

2,945,762

SUPERSENSITIZATION OF PHOTOGRAPHIC EMULSIONS USING TRIAZINES

Filed Oct. 12, 1955

**Fig. 1**



A=3,3'-DIETHYLOXATHIADICARBOCYANINE IODIDE  
B=3,3'-DIETHYLOXATHIADICARBOCYANINE IODIDE WITH 4,4'-  
BIS[4-(4'-SULFOANILINO)-6- $\beta$ -HYDROXYETHYLAMINO-S-  
TRIAZIN-2-YLAMINO] STILBENE-2,2'-DISULFONIC ACID

**Fig. 2**



C=3,3'-DIETHYLOXATHIADICARBOCYANINE IODIDE WITH  
4,4'-BIS(4,6-DIANILINO-S-TRIAZIN-2-YLAMINO) STILBENE-  
2,2'-DISULFONIC ACID

**Fig. 3**



D=3,3'-DIETHYLOXATHIADICARBOCYANINE IODIDE WITH 4,4'-  
BIS(4-PHOENOXY-6- $\beta$ -HYDROXYETHYLAMINO-S-TRIAZIN-2-  
YLAMINO) STILBENE-2,2'-DISULFONIC ACID

*Burt H. Carroll  
Jean E. Jones  
John Spence*  
INVENTORS

*BY*  
*Daniel I. Mayne*  
*Lawrence H. Willis*  
ATTORNEYS

1

2,945,762

## SUPERSENSITIZATION OF PHOTOGRAPHIC EMULSIONS USING TRIAZINES

Burt H. Carroll, Jean E. Jones, and John Spence, Rochester, N.Y., assignors to Eastman Kodak Company, Rochester, N.Y., a corporation of New Jersey

Filed Oct. 12, 1955, Ser. No. 540,052

16 Claims. (Cl. 96—100)

This invention relates to photographic silver halide emulsions useful in color photography and photographic silver halide emulsions containing certain dicarbocyanine dyes, and as supersensitizers therefor, bis-triazinylaminostilbene compounds.

It is known in the art of making photographic emulsions that certain dyes of the cyanine class alter the sensitivity of photographic emulsions of the gelatino-silver-halide kind, when the dyes are incorporated in the emulsions. It is also known that the sensitization produced by a given dye varies somewhat with the type of emulsion in which the dye is incorporated. Furthermore, the sensitization of a given emulsion by a given dye may be altered by varying the conditions in the emulsion. For example, the sensitization may be increased by increasing the silver ion concentration or decreasing the hydrogen ion concentration (i.e., increasing the alkalinity) or both. Thus, sensitization can be increased by bathing plates, coated with a spectrally sensitized emulsion, in water or in aqueous solutions of ammonia. Such a process of altering the sensitivity of a sensitized emulsion by increasing the silver ion concentration and/or by decreasing the hydrogen ion concentration is commonly called "hypersensitization." Hypersensitized emulsions have generally poor keeping qualities.

We have now found another means of altering the sensitivity in emulsions containing certain dicarbocyanine dyes. Since the conditions in the emulsions, i.e., the hydrogen ion and/or the silver ion concentration undergo little or no change in our method, we shall designate our method as a kind of supersensitization.

It is, therefore, an object of our invention to provide photographic emulsions containing certain dicarbocyanine dyes, and as supersensitizers therefore, bis-triazinylaminostilbene compounds. Another object is to provide a means for preparing these supersensitized emulsions. Still another object is to provide photographic emulsions containing bis-triazinylaminostilbene compounds which are especially useful in color photography. Other objects will become apparent from a consideration of the following description and examples.

The dicarbocyanine dyes which are useful in practicing our invention can advantageously be represented by the following general formula:



wherein R and R<sub>1</sub> each represents an alkyl group (such as methyl, ethyl,  $\beta$ -hydroxyethyl, carboxymethyl,  $\beta$ -carboxyethyl, carbomethoxymethyl, carbethoxymethyl, etc., n represents a positive integer of from 1 to 2, X represents an acid radical, such as chloride, iodide, bromide, perchlorate, p-toluenesulfonate, benzenesulfonate, ethylsulfate, methylsulfate, etc., Z represents the non-metallic atoms necessary to complete a heterocyclic nucleus containing from 5 to 6 atoms in the heterocyclic ring, e.g.,

2

a heterocyclic nucleus of the benzothiazole series (e.g., benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 4-phenylbenzothiazole, 5-phenylbenzothiazole, 4-methoxybenzothiazole, 5-methoxybenzothiazole, 6-methoxybenzothiazole, 6-iodobenzothiazole, 5-iodobenzothiazole, 4-ethoxybenzothiazole, 5-ethoxybenzothiazole, 5,6-dimethylbenzothiazole, 5-hydroxybenzothiazole, 6-hydroxybenzothiazole, etc.), a heterocyclic nucleus of the naphthothiazole series (e.g.,  $\alpha$ -naphthothiazole,  $\beta$ -naphthothiazole, 7-methoxy- $\alpha$ -naphthothiazole, 8-methoxy- $\alpha$ -naphthothiazole, 5-methoxy- $\beta$ -naphthothiazole, 5-ethoxy- $\alpha$ -naphthothiazole, etc.), a heterocyclic nucleus of the benzoselenazole series (e.g., benzoselenazole, 5-chlorobenzoselenazole, 6-methoxybenzoselenazole, 5-methoxybenzoselenazole, etc.), a heterocyclic nucleus of the naphthoselenazole series (e.g.,  $\alpha$ -naphthoselenazole,  $\beta$ -naphthoselenazole, etc.), a heterocyclic nucleus of the benzoxazole series (e.g., benzoxazole, 5-hydroxybenzoxazole, 6-hydroxybenzoxazole, 5-chlorobenzoxazole, 5-methoxybenzoxazole, 6-methoxybenzoxazole, 5-phenylbenzoxazole, 5-bromobenzoxazole, etc.), and a heterocyclic nucleus of the naphthoxazole series (e.g.,  $\alpha$ -naphthoxazole,  $\beta$ -naphthoxazole, etc.), and Z<sub>1</sub> represents the non-metallic atoms necessary to complete a heterocyclic nucleus selected from the group consisting of a heterocyclic nucleus of the benzoxazole series (e.g., such as those defined by Z above), a heterocyclic nucleus of the naphthoxazole series (e.g., such as those defined by Z above), a heterocyclic nucleus of the benzoselenazole series (e.g., such as those defined by Z above), a heterocyclic nucleus of the naphthoselenazole series (e.g., such as those defined by Z above), a heterocyclic nucleus of the naphthothiazole series (e.g., such as those defined by Z above), a heterocyclic nucleus of the 2-quinoline series (e.g., 2-quinoline, 6-methyl-2-quinoline, 7-methyl-2-quinoline, 8-methyl-2-quinoline, 6-chloro-2-quinoline, 8-chloro-2-quinoline, 4-chloro-2-quinoline, 5-ethoxy-2-quinoline, 6-ethoxy-2-quinoline, 7-ethoxy-2-quinoline, 6-hydroxy-2-quinoline, 7-hydroxy-2-quinoline, 6-methoxy-2-quinoline, etc.), a heterocyclic nucleus of the 4-quinoline series (e.g., 4-quinoline, 6-methoxy-4-quinoline, 7-methyl-4-quinoline, 8-methyl-4-quinoline, etc.), a heterocyclic nucleus of the benzimidazole series (e.g., benzimidazole, 5-chlorobenzimidazole, 5,6-dichlorobenzimidazole, 1,7-trimethylenebenzimidazole, etc.), and a heterocyclic nucleus of the 5,6-benzoquinoline series (e.g., 5,6-benzo-2-quinoline, etc.).

45 The bis-triazinylaminostilbene compounds useful in practicing our invention have been previously employed in the art as fluorescent agents and as bleaching (optical) agents, and hence are widely known substances. Especially useful compounds of this class comprise those compounds represented by the following general formula:

II.



wherein R<sub>6</sub>, R<sub>7</sub>, R<sub>2</sub>, and R<sub>3</sub> each represents a hydrogen atom, or a substituent group, such as hydroxyl, aryloxyl (e.g., phenoxy, o-toloxyl, p-sulfophenoxy, etc.), alkoxy (e.g., methoxy, ethoxy, etc.), a halogen atom (e.g., chlorine, bromine, etc.), a heterocyclic radical (e.g., morpholinyl, piperidyl, etc.), an alkylthio group (e.g., methylthio, ethylthio, etc.), an arylthio group (e.g., phenylthio, tolylthio, etc.), a heterocyclylthio group (e.g., benzothiazylthio, etc.), an amino group, an alkylamino group

(e.g., methylamino, ethylamino, propylamino, dimethylamino, diethylamino, dodecylamino, cyclohexylamino,  $\beta$ -hydroxyethylamino, di- $\beta$ -hydroxyethylamino,  $\beta$ -sulfoethylamino, etc.), an arylamino group (e.g., anilino, o-, m-, and p-sulfoanilino, o-, m-, and p-chloroanilino, o-, m-, and p-anisylamino, o-, m-, and p-toluidino, o-, m-, and p-carboxyanilino, hydroxyanilino, sulfonaphthylamino, o-, m-, and p-aminoanilino, p-acetamidoanilino, etc.), etc., and R<sub>4</sub> and R<sub>5</sub> each represents a hydrogen atom or a water-solubilizing group, such as sulfo, carboxyl, etc. (as well as alkali metal or amine salts of such groups). Many of the compounds represented by Formula II above are known substances, and methods for preparing these compounds are well known. Listed below are representative compounds selected from those represented by Formula II, although our invention is not limited in any sense to these particular compounds. While the structural formulas are included for only the first three compounds, it is to be understood that the same numbering system is employed throughout the specification.



- (4) 4,4'-bis[4-(4'-sulfoanilino)-6-( $\beta$ -hydroxyethylamino)-s-triazin-2-ylamino]stilbene-2,2'-disulfonic acid
- (5) 4,4'-bis[4,6-dianilino-s-triazinyl-2-ylamino]stilbene-2,2'-disulfonic acid
- (6) 4,4'-bis[4-phenoxy-6-( $\beta$ -hydroxyethylamino)-s-triazin-2-ylamino]stilbene-2,2'-disulfonic acid
- (7) 4,4'-bis(4,6-dianilino-s-triazin-2-ylamino)stilbene
- (8) 4,4'-bis(4,6-dihydroxy-s-triazin-2-ylamino)stilbene-2,2'-disulfonic acid
- (9) 4,4'-bis(4-anilino-6-hydroxy-s-triazin-2-ylamino)stilbene-2,2'-disulfonic acid

- (10) 4,4'-bis[4-(2'-chloroanilino)-6-hydroxy-s-triazin-2-ylamino]stilbene-2,2'-disulfonic acid
- (11) 4,4'-bis[4-(5'-sulfonaphthylamino)-6-hydroxy-s-triazin-2-ylamino]stilbene-2,2'-disulfonic acid
- (12) 4,4'-bis[4-n-dodecylamino-6-( $\beta$ -sulfoethylamino)-s-triazin-2-ylamino]stilbene-2,2'-disulfonic acid
- (13) 4,4'-bis[4-N-morpholiny-6-(4'-sulfoanilino)-s-triazin-2-ylamino]stilbene-2,2'-disulfonic acid
- (14) 4,4'-bis[4,6-di(N-morpholiny)-s-triazin-2-ylamino]stilbene-2,2'-disulfonic acid
- (15) 4,4'-bis-{4-[4'-(5'-keto-3'-methyl-2'-pyrazolin-1'-yl)-anilino]-6-hydroxy-s-triazin-2-ylamino}stilbene-2,2'-disulfonic acid
- (16) 4-[4-ethylamino-6-(di- $\beta$ -hydroxyethylamino)-s-triazin-2-ylamino]-4'-[4-methylamino-6-( $\beta$ -hydroxyethylamino)-s-triazin-2-ylamino]stilbene-2,2'-disulfonic acid
- (17) 4-[4-methylamino-6-( $\beta$ -hydroxyethylamino)-s-triazin-2-ylamino]-4'-[4-ethylamino-6-(2'-anisidino)-s-triazin-2-ylamino]stilbene-2,2'-disulfonic acid
- (18) 4-[4-ethylamino-6-( $\beta$ -hydroxyethylamino)-s-triazin-2-ylamino]-4'-[4,6-diamino-s-triazin-2-ylamino]stilbene-2,2'-disulfonic acid
- (19) 4,4'-bis[4-chloro-6-di( $\beta$ -hydroxyethylamino)-s-triazin-2-ylamino]stilbene-2,2'-disulfonic acid
- (20) 4,4'-bis[4-anilino-6-( $\beta$ -hydroxyethylamino)-s-triazin-2-ylamino]stilbene-2,2'-disulfonic acid
- (21) 4,4'-bis[4-(4'-acetamidoanilino)-6-( $\beta$ -hydroxyethylamino)-s-triazin-2-ylamino]stilbene-2,2'-disulfonic acid
- (22) 4,4'-bis[4-amino-6-(3'-carboxyphenylamino)-s-triazin-2-ylamino]stilbene-2,2'-disulfonic acid
- (23) 4-[4-phenoxy-6-( $\beta$ -hydroxyethylamino)-s-triazin-2-ylamino]-4'-[4-chloro-6-di( $\beta$ -hydroxyethylamino)-s-triazin-2-ylamino]stilbene-2,2'-disulfonic acid
- (24) 4,4'-bis[4-ethylthio-6-( $\beta$ -hydroxyethylamino)-s-triazin-2-ylamino]stilbene-2,2'-disulfonic acid
- (25) 4,4'-bis[4-phenylthio-6-( $\beta$ -hydroxyethylamino)-s-triazin-2-ylamino]stilbene-2,2'-disulfonic acid
- (26) 4,4'-bis(s-triazin-2-ylamino)stilbene-2,2'-disulfonic acid
- (27) 4,4'-bis(4-hydroxy-6-amino-s-triazin-2-ylamino)stilbene-2,2'-disulfonic acid
- (28) 4,4'-bis(4-chloro-6-trimethylolmethylamino-s-triazin-2-ylamino)stilbene-2,2'-disulfonic acid

Compounds of the above type which can advantageously be employed in practicing our invention have been described in one or more of the following representative patents:

|       |           |               |
|-------|-----------|---------------|
| U.S.: |           |               |
|       | 2,171,427 | Aug. 29, 1939 |
|       | 2,473,475 | June 14, 1949 |
|       | 2,595,030 | Apr. 29, 1952 |
|       | 2,660,578 | Nov. 24, 1953 |
| Br.:  |           |               |
|       | 595,065   | Nov. 26, 1947 |
|       | 623,849   | May 24, 1949  |
|       | 624,051   | May 26, 1949  |
|       | 624,052   | May 26, 1949  |
|       | 678,291   | Sept. 3, 1952 |
|       | 681,642   | Oct. 29, 1952 |
|       | 705,406   | Mar. 10, 1954 |

These products have been previously employed in the textile field, and are sold under such trade names as Leucophor B, Calcofluor White MR, Tinopal (SP, WR, BV277, 2B, GS, NG), Blancofor SC, Hiltamine (BSP, N, Sol, 6T6), and the like.

According to our invention, we incorporate one or more of the dicarbocyanine dyes represented by Formula I above with one or more s-triazinylaminostilbene compounds, such as those represented by Formula II above. Our invention is particularly directed to the ordinarily employed gelatino-silver-halide emulsions. However, our supersensitizing combinations can be employed in silver halide emulsions in which the carrier is other than gelatin, e.g., a resinous substance or cellulosic material which has no deteriorating effect on the light-sensitive materials. The dicarbocyanine dyes and s-triazinylaminostilbene compounds can be employed in various concentrations depending upon the effects desired.

Ordinarily, the optimum or near optimum concentration of the dicarbocyanine dyes which we employ in practicing our invention is of the order of from 0.010 to 0.30 g. per mol. of silver halide in the emulsion.

The s-triazinylaminostilbene compounds which we employ in our invention can advantageously be employed at a concentration of from about 0.03 to 10.0 g. per mol. of silver halide in the emulsion.

In general, the ratio of concentration of dicarbocyanine dye s-triazinylaminostilbene compound can vary rather widely in our combinations, e.g., from 1:1 to 1:300 (by weight) in many cases.

The methods of incorporating sensitizing dyes in silver halide emulsions are well known to those skilled in the art. The s-triazinylaminostilbene compounds can be directly dispersed in the emulsions, or they can be dissolved in water (or an organic solvent, such as methanol, ethanol, etc., where the water-solubility is not sufficiently great) and added in the form of their solutions. While the dicarbocyanine dyes can be directly dispersed in the emulsions, it is convenient to add the same in the form of solutions in appropriate solvents. Methanol, ethanol, pyridine, and the like have proven satisfactory for many of the dyes of Formula I. Mixtures of solvents, e.g., pyridine diluted with methanol or acetone, can also be used. The dicarbocyanine dyes and s-triazinylaminostilbene compounds are dispersed in the finished emulsions and should be uniformly distributed throughout the emulsions. The following procedure is satisfactory: Stock solutions of the dicarbocyanine dyes and stilbene compounds are prepared by dissolving the same

in appropriate solvents as described above. Then, to the flowable gelatino-silver-halide emulsion, the desired amounts of the stock solution of one of the dyes (or stilbene compounds) are slowly added, while stirring the emulsion. Stirring is continued until the dye is thoroughly incorporated in the emulsion. Then the desired amount of the stock solution of the stilbene compound (or dye, if stilbene compound has been added first) is slowly added to the emulsion, while stirring. Stirring is continued until the second solution is thoroughly incorporated. The supersensitized emulsion can then be coated out on a suitable support, such as glass, cellulose derivative film, resin film, or paper, to a suitable thickness and allowed to dry. The details of such coating methods are well known to those skilled in the art. The foregoing procedures and proportions are to be regarded only as illustrative. Clearly, our invention is directed to any silver halide emulsion containing a combination of the aforesaid dicarbocyanine dyes and s-triazinylaminostilbene compounds whereby a supersensitizing effect is obtained.

The following examples will serve to illustrate further the manner of practicing our invention.

In Table I below, to different portions of the same batch of photographic gelatino-silver-halide emulsion were added (1) a dicarbocyanine dye, such as those represented by Formula I above, and (2) a combination of the dicarbocyanine dye and a bis(s-triazin-2-ylamino) stilbene (in neutral aqueous solution). Then the emulsions were held at about 40° C. for a short time and coated on a support, chill set, and dried. After exposure through a Wratten No. 25 filter, i.e., a filter which transmits substantially no light of wavelength shorter than about 580 mu (Examples 1 to 14 and 17 to 31) or a Wratten No. 12 filter, i.e., a filter which transmits substantially no light of wavelength shorter than about 495 mu, (Examples 15 and 16) in an Eastman Type IB sensitometer, the film strips were processed for 3 minutes in a developer having the following composition:

|                                |    |      |
|--------------------------------|----|------|
| N-methyl-p-aminophenol sulfate | g. | 2.0  |
| Hydroquinone                   | g. | 8.0  |
| Sodium sulfite (desiccated)    | g. | 90.0 |
| Sodium carbonate (monohydrate) | g. | 52.5 |
| Potassium bromide              | g. | 5.0  |
| Water to make 1 liter.         |    |      |

The speed (red or minus blue), gamma and fog for each of the coatings was then measured. The results are recorded in Table I.

Table I

| Example | Sensitizing Dye & Addenda (g./mol. AgX)                                    | Red or Minus Blue Light Exposure |       |     |
|---------|----------------------------------------------------------------------------|----------------------------------|-------|-----|
|         |                                                                            | 30/E Speed                       | Gamma | Fog |
| 1.....  | (a) 3,3'-diethylselenadicarbocyanine bromide (.075)                        | 20                               | 2.3   | .22 |
|         | (b) dye (a) (.075) plus Calcofluor White MR <sup>1</sup> (.13)             | 25                               | 2.0   | .31 |
| 2.....  | (c) 3,3'-diethylxanthiadicarbocyanine iodide (.050)                        | 3.7                              | 1.3   | .06 |
|         | (d) dye (c) (.050) plus compound 4 (3.0)                                   | 20.5                             | 2.7   | .06 |
| 3.....  | (e) dye (c) (.050) plus compound 1 (3.0)                                   | 6.7                              | 2.4   | .05 |
| 4.....  | (f) dye (c) (.050) plus compound 5 (3.0)                                   | 24.5                             | 2.9   | .05 |
| 5.....  | (g) dye (c) (.050) plus compound 6 (3.0)                                   | 22.                              | 2.9   | .06 |
| 6.....  | (h) dye (c) (.050) plus compound 2 (3.0)                                   | 27.5                             | 2.8   | .06 |
| 7.....  | (i) dye (c) (.0375)                                                        | 32                               | 3.0   | .06 |
|         | (j) dye (c) (.0375) plus compound 6 (2.5)                                  | 111                              | 2.1   | .06 |
| 8.....  | (k) dye (c) (.050)                                                         | nil                              | nil   | .05 |
|         | (l) dye (c) (.050) plus Calcofluor White MR <sup>1</sup> (3.0)             | 34.5                             | 2.4   | .06 |
| 9.....  | (m) dye (a) (.050)                                                         | 5.1                              | .73   | .07 |
|         | (n) dye (a) (.050) plus Calcofluor White MR <sup>1</sup> (3.0)             | 16.5                             | 2.4   | .06 |
| 10..... | (o) dye (c) (.050)                                                         | 4.65                             | 1.5   | .06 |
|         | (p) dye (c) (.050) plus Calcofluor White MR <sup>1</sup> (3.0)             | 11.9                             | 2.0   | .06 |
| 11..... | (q) dye (c) (.050)                                                         | 4.25                             | 1.3   | .06 |
|         | (r) dye (c) (.050) plus Calcofluor White MR <sup>1</sup> (3.0)             | 13.7                             | 2.3   | .07 |
| 12..... | (s) 3-ethyl-3'-β-hydroxyethylxanthiadicarbocyanine iodide (.050)           | 11.9                             | 2.8   | .06 |
|         | (t) dye (s) (.050) plus Calcofluor White MR <sup>1</sup> (3.0)             | 22.0                             | 2.3   | .07 |
| 13..... | (u) 3,3'-diethyl-5-phenyloxanthiadicarbocyanine-p-toluene-sulfonate (.050) | nil                              | nil   | .06 |
|         | (v) dye (u) (.050) plus Calcofluor White MR <sup>1</sup> (3.0)             | 4.15                             | 1.3   | .08 |

Table I—Continued

| Example | Sensitizing Dye & Addenda (g./mol. AgX)                                                                   | Red or Minus Blue Light Exposure |       |     |
|---------|-----------------------------------------------------------------------------------------------------------|----------------------------------|-------|-----|
|         |                                                                                                           | 30/E Speed                       | Gamma | Fog |
| 14.     | (w) 3-ethyl-3'- $\beta$ -hydroxyethyl-5-phenyloxathiadcarbocyanine bromide (.050)                         | 4.55                             | 1.5   | .06 |
|         | (x) dye (w) (.050) plus Calcofluor White M.R. <sup>1</sup> (3.0)                                          | 9.25                             | 1.9   | .08 |
| 15.     | (y) 3,3'-diethyloxadcarbocyanine iodide (.050)                                                            | 7.7                              | 2.0   | .06 |
|         | (z) dye (y) plus compound 27 (.30)                                                                        | 19.0                             | 2.1   | .06 |
| 16.     | (a') 3,3'-diethyl-5,5'-diphenyloxadcarbocyanine perchlorate (.050)                                        | 3.8                              | 1.4   | .06 |
|         | (b') dye (a') (.050) plus compound 27 (.30)                                                               | 9.1                              | 2.1   | .07 |
| 17.     | (c') 3,3'-diethyl-6,7,6',7'-dibenzoxadcarbocyanine iodide (.050)                                          | 4.2                              | 1.3   | .06 |
|         | (d') dye (c') (.050) plus compound 27 (.30)                                                               | 6.0                              | 1.5   | .07 |
| 18.     | (e') 3,3'-dimethyl-4,5,4',5'-dibenzothiadcarbocyanine chloride (.050)                                     | .93                              | .79   | .06 |
|         | (f') dye (e') (.050) plus compound 27 (.30)                                                               | 4.1                              | 1.4   | .07 |
| 19.     | (g') 3,3'-diethyl-6,7,6',7'-dibenzothiadcarbocyanine iodide (.050)                                        | 2.6                              | 1.6   | .05 |
|         | (h') dye (g') (.050) plus compound 27 (.30)                                                               | 4.4                              | 1.1   | .06 |
| 20.     | (i') 3,1'-diethyl-5,6-benzoselena-2'-dcarbocyanine iodide (.050)                                          | .97                              | .66   | .07 |
|         | (j') dye (i') (.050) plus compound 27 (.30)                                                               | 3.3                              | 1.9   | .06 |
| 21.     | (k') 3,3'-diethyl-4,5,6',7'-dibenzoselena-2'-dcarbocyanine iodide (.050)                                  | 2.4                              | 1.8   | .05 |
|         | (l') dye (k') (.050) plus compound 27 (.30)                                                               | 3.5                              | .98   | .06 |
| 22.     | (m') 3,3'-diethyl-6,7-benzoselena-2'-dcarbocyanine iodide (.050)                                          | 2.8                              | 1.8   | .05 |
|         | (n') dye (m') (.050) plus compound 27 (.30)                                                               | 3.5                              | .9    | .06 |
| 23.     | (o') 3,3'-diethyl-4,5,6',7'-dibenzothiadcarbocyanine iodide (.050)                                        | 1.6                              | 1.2   | .06 |
|         | (p') dye (o') (.050) plus compound 27 (.30)                                                               | 3.3                              | 1.0   | .06 |
| 24.     | (q') 3,1'-diethyl-6,7-benzothiadcarbocyanine iodide                                                       | nll                              | nll   | .06 |
|         | (r') dye (q') (.050) plus compound 27 (.30)                                                               | 3.9                              | 1.6   | .06 |
| 25.     | (s') 3,1'-diethyl-4,5,6',7'-dibenzothia-2'-dcarbocyanine iodide (.050)                                    | nll                              | nll   | .13 |
|         | (t') dye (s') (.050) plus compound 27 (.30)                                                               | 4.2                              | 1.1   | .10 |
| 26.     | (u') 3,1'-diethyl-6,7-benzothia-4'-dcarbocyanine iodide (.050)                                            | nll                              | nll   | .09 |
|         | (v') dye (u') (.050) plus compound 27 (.30)                                                               | 1.6                              | 1.4   | .08 |
| 27.     | (w') 3,3'-diethyl-4,5,6',7'-dibenzothiadcarbocyanine iodide (.050)                                        | 3.2                              | 1.8   | .05 |
|         | (x') dye (w') (.050) plus compound 27 (.30)                                                               | 5.2                              | 1.2   | .07 |
| 28.     | (y') (3-ethyl-2-benzothiazole) (3-ethyl-1,7-trimethylene-2-benzimidazol)pentamethinecyanine iodide (.050) | 8.2                              | 1.9   | .05 |
|         | (z') dye (y') (.050) plus compound 27 (.30)                                                               | 11.1                             | 2.3   | .06 |
| 29.     | (a') 3,3'-diethyl-6,7-benzothiadcarbocyanine iodide (.050)                                                | 2.2                              | 1.4   | .06 |
|         | (b') dye (a') (.050) plus compound 27 (.30)                                                               | 5.2                              | 1.3   | .06 |
| 30.     | (c') 1',3-diethyl-4,5-benzothia-2'-dcarbocyanine iodide (.050)                                            | 3.8                              | 2.3   | .07 |
|         | (d') dye (c') (.050) plus compound 27 (.30)                                                               | 8.4                              | 1.9   | .07 |
| 31.     | (e') 3,3'-diethyl-4,5,4',5'-dibenzoselena-2'-dcarbocyanine iodide (.050)                                  | 1.7                              | 1.2   | .06 |
|         | (f') dye (e') (.050) plus compound 27 (.30)                                                               | 4.4                              | 2.0   | .06 |

<sup>1</sup> = Calcofluor White M.R. is a bis(*s*-triazin-2-ylamino)stilbene-2,2'-disulfonic acid (as sodium salt).

In the above table, the coatings of Examples 2 to 6 were made from the same batch of gelatino-silver-bromide emulsion, the coatings of Example 1 were made from the same batch of gelatino-silver-chlorobromide emulsion, the coatings of Example 7 were made from the same batch of gelatino-silver-chlorobromide emulsion, the coatings of Examples 8 and 9 were made from the same batch of gelatino-silver-bromide emulsion, the coatings of Example 10 were made from the same batch of gelatino-silver-bromide emulsion, the coatings of Examples 11 to 14 were made from the same batch of gelatino-silver-bromide emulsion, the coatings of Examples 15 and 16 were made from the same batch of gelatino-silver-bromide emulsion, and the coatings of Examples 17 to 31 were made from the same batch of gelatino-silver-bromide emulsion. No measurements for the stilbene compounds alone are given in the table, since numerous coatings at the concentrations used in the table have shown that these stilbene compounds when employed alone have no positive measurable effect (sensitometrically).

Our invention is primarily directed to the ordinarily employed gelatino-silver-halide developing-out emulsions, e.g., gelatino-silver-chloride, -chlorobromide, -chloroiodide, -chlorobromiodide, -bromide and -bromiodide developing-out emulsions. Emulsions which form the latent image mostly inside the silver halide grains, such as the emulsions set forth in U.S. Patent 2,456,956, dated December 21, 1948, can also be employed in practicing our invention.

The emulsions prepared in accordance with our invention can be coated in the usual manner on any suitable support, e.g., glass, cellulose nitrate film, cellulose acetate film, polyvinylacetal resin film, paper or metal.

Photographic silver halide emulsions, such as those listed above, containing the supersensitizing combinations of our invention can also contain such addenda as chemical sensitizers, e.g., sulfur sensitizers (e.g., allyl thiocarbamide, thiourea, allylisothiocyanate, cystine, etc.), various gold compounds (e.g., potassium chloroaurate, auric trichloride, etc.) (see U.S. Patents 2,540,085; 2,597,856 and 2,597,915), various palladium compounds, such as palladium chloride (U.S. 2,540,086), potassium chloropalladate (U.S. 2,598,079), etc., or mixtures of such sensitizers; anti-foggants, such as ammonium chloroplatinate (U.S. 2,566,245), ammonium chloroplatinite (U.S. 2,566,263), benzotriazole, nitrobenzimidazole, 5-nitroindazole, benzidine, mercaptans, etc. (see Mees—“The Theory of the Photographic Process,” Macmillan Pub., page 460), or mixtures thereof; hardeners, such as formaldehyde (U.S. 1,763,533), chrome alum (U.S. 1,763,533), glyoxal (U.S. 1,870,354), dibromacrolein (Br. 406,750), etc.; color couplers, such as those described in U.S. Patent 2,423,730, Spence and Carroll U.S. Patent 2,640,776, etc.; or mixtures of such addenda. Dispersing agents for color couplers, such as those set forth in U.S. Patents 2,322,027 and 2,304,940, can also be employed in the above-described emulsions.

Such silver halide emulsions can also contain thiazolidones or other ultraviolet absorbing compounds, such as those described in the copending application Serial No. 419,239, filed March 29, 1954 in the name of G. W. Sawdey, now U.S. Patent 2,739,888, issued March 27, 1956. While certain emulsion addenda, such as certain ultraviolet compounds, and certain color-forming compounds cause de-sensitization or un-sensitizing effects, it has been found that the new combinations of our invention largely overcome such effects. Typical color-form-

ing compounds which can be so employed include those in U.S. Patent 2,322,027 and the following:

Coupler:

- (1) 1-hydroxy-2-[ $\delta$ -(2',4' - di - tert.amylphenoxy)-n-butyl]-naphthamide (U.S. Patent 2,474,293)
- (2) 1-hydroxy - 4 - phenylazo-4'-(p-tert.-butylphenoxy)-3-naphthanilide (U.S. Patent 2,521,908)
- (3) 2-(2,4-di-tert.amylphenoxyacetamino) - 4,6-dichloro-5-methyl phenol (Graham U.S. application Serial No. 285,544, now U.S. Patent 2,725,291)
- (4) 2-( $\alpha$ -2,4-di-tert.amylphenoxy - n-butylamino)-4,6-dichloro-5-methyl phenol
- (5) 6-{ $\alpha$ -{4-[ $\alpha$ -(2,4 - di - tert.amylphenoxy)butyramido] - phenoxy}acetamido}-2,4 - dichloro - 3 - methyl phenol
- (6) 2-[3' - (2',4' - di-tert.amylphenoxy) - acetamido]-benzamido-4-chloro-5-methyl phenol
- (7) 1-(2',4',6'-trichlorophenyl)-3-[3'-(2'',4'' - di-tert.-amylphenoxyacetamido) - benzamido]-5-pyrazolone (U.S. Patent 2,600,788)
- (8) 1-(2',4',6'-trichlorophenyl)-3 - [3' - 2'',4''-di-tert.amylphenoxyacetamido) - benzamido]-4-(p-methoxyphenoxy)-5-pyrazolone
- (9) N-(4-benzoylacetamino)benzenesulfonyl) - N-( $\gamma$ -phenylpropyl)-p-toluidine (U.S. Patent 2,298,443)
- (10)  $\alpha$ -o-Methoxybenzoyl -  $\alpha$  - chloro-4-[ $\alpha$ -(2,4-di-tert. - amylphenoxy) - n-butylamido] - acetanilide (McCrossen U.S. application Serial No. 295,806, now U.S. Patent 2,728,658, issued December 27, 1955)
- (11)  $\alpha$ -{3-[ $\alpha$ -(2,4 - di - tert.amylphenoxy) acetamido-benzoyl]-2-methoxyacetanilide}
- (12) 3-benzoylacetamido - 4 - methoxy-2',4'-di-tert.-amylphenoxy acetanilide
- (13) 4-benzoylacetamido - 3 - methoxy-2',4'-di-tert.-amylphenoxy acetanilide

The following examples will serve to illustrate the beneficial effects of our new supersensitizing combinations when employed in multilayer photographic emulsion layers containing incorporated color-forming compounds.

EXAMPLE 32

A photographic gelatino-silver-chlorobromide emulsion containing a coupler dispersion of a color-forming compound, such as coupler No. 5 above, and a thiazolidone ultraviolet absorbing compound, such as 5-benzal-3-n-cetyl-2-phenylimino-4-thiazolidone, was sensitized with dye (c) of Table I (.075 g./mol. AgX). To one portion of such sensitized emulsion was added Leucophor B (10 g./mol. AgX) while none was added to the remainder. These were then coated on separate baryta-coated paper supports and the coatings exposed on a sensitometer and reversal processed by first developing for 6 minutes in a developer having the following composition:

G.

|                                   |      |
|-----------------------------------|------|
| Calgon (sodium hexametaphosphate) | 2.0  |
| 4-N-methylaminophenol sulfate     | .9   |
| Hydroquinone                      | 2.35 |
| Sodium sulfite (anhyd.)           | 8.0  |
| Sodium carbonate (anhyd.)         | 10.0 |
| Potassium bromide                 | .55  |
| Sodium chloride                   | .20  |
| 5-methylbenzotriazole             | .02  |
| Water to make 1 liter.            |      |

After treatment in a conventional stop bath and washing, the coatings were re-exposed with a photoflood and color developed in a bath of the following composition:

|                                   |    |      |
|-----------------------------------|----|------|
| Benzyl alcohol                    | cc | 15   |
| Calgon (sodium hexametaphosphate) | g  | 2.0  |
| Sodium carbonate (anhyd.)         | g  | 20.0 |
| Sodium hydroxide                  | g  | 2.0  |
| Sodium sulfite (anhyd.)           | g  | 2.0  |
| Developer <sup>1</sup>            | g  | 4.0  |

75

|                             |   |     |
|-----------------------------|---|-----|
| Hydroxylamine hydrochloride | g | 4.0 |
| Potassium bromide           | g | .1  |
| Water to make 1 liter.      |   |     |

|   |                                                                             |
|---|-----------------------------------------------------------------------------|
| 5 | 1-N-ethyl-N- $\beta$ -methanesulfonamidoethyl - 3 - methyl-4-amino-aniline. |
|---|-----------------------------------------------------------------------------|

After treatment in a conventional stop bath, the coatings were bleached with ferricyanide and bromide and fixed in a bath of the type described in U.S. Patent 2,706,687. The relative red and minus blue speeds (density 0.3 fog) for each of the coatings was measured. The results follow:

|                          | Red Speed | Minus Blue Speed |
|--------------------------|-----------|------------------|
| 15                       |           |                  |
| dye (c) alone            | .81       | .86              |
| dye (c) plus Leucophor B | 2.20      | .85              |

The coatings described in the following examples were prepared in substantially the same manner as those set forth in Example 32 above. However, no ultraviolet-absorbing compound was employed and the emulsions were coated on a cellulose acetate support instead of paper. Either Leucophor B or Calcofluor White MR (both, 10 g./mol. AgX) was employed as shown in Table II below. To measure the anti-unsensitizing effect of these stilbene compounds, series of coatings were held at 40° C. for 30 minutes and 60 minutes, respectively, before coating for comparison with a series of fresh coatings (0' holding). The coatings were then exposed in the usual manner and color developed in a developer having the following composition:

|                                |    |      |
|--------------------------------|----|------|
| Water (70-75° F.)              | cc | 800  |
| Calgon                         | g  | 2.0  |
| Sodium sulfate (anhydrous)     | g  | 4.0  |
| Developer <sup>1</sup>         | g  | 3.0  |
| Sodium carbonate (monohydrate) | g  | 20.0 |
| Potassium bromide              | g  | 2.0  |
| Water to make 1 liter.         |    |      |

40 1-2-amino-5-diethylamino toluene hydrochloride.

The coating was then rinsed, fixed, bleached with potassium dichromate, etc., in the usual manner. The results are given in the following table.

45

Table II

| Example    | Addenda             | Holding Time | Red Speed | Minus Blue Speed |
|------------|---------------------|--------------|-----------|------------------|
| 50 33. (a) | none                | 0'           | nil       | .80              |
| 33. (b)    | Leucophor B         | 0'           | 1.11      | .87              |
| 34.        | Calcofluor White MR | 0'           | 1.30      | .80              |
| 35. (a)    | none                | 30'@40° C.   | nil       | .88              |
| 35. (b)    | Leucophor B         | 30'@40° C.   | .62       | .88              |
| 36.        | Calcofluor White MR | 30'@40° C.   | .98       | .81              |
| 37. (a)    | none                | 60'@40° C.   | nil       | .86              |
| 37. (b)    | Leucophor B         | 60'@40° C.   | .44       | .91              |
| 38.        | Calcofluor White MR | 60'@40° C.   | .69       | .70              |

In exactly the manner described for the coating of Table I, dye (c) (.050 g./mol. AgX) was incorporated in an ordinary gelatino-silver-bromide emulsion and together (at the same concentration) with compound 7 (8.0 g./mol. AgX). The relative speed (red), gamma and fog are given for each of these coatings:

| 65 | Example 39              | Relative Speed | Gamma | Fog |
|----|-------------------------|----------------|-------|-----|
|    | dye (c) alone           | 100            | 4.5   | .06 |
|    | dye (c) plus compound 7 | 245            | 5.3   | .06 |

70 While we have found that tricarbocyanine dyes corresponding to the dicarbocyanine dyes of Formula I (e.g., 3,3'-diethylthiatricarbocyanine iodide) can sometimes be used to advantage in combination with the compounds of Formula II (e.g., with compound 4 or Calcofluor White MR), generally these combinations do not

## 11

provide as advantageous results as those described above. A set of coatings of an ordinary gelatino-silver-bromide emulsion was prepared as described above for the coatings of Table I. The results follows:

| Example 40                                         | Red<br>(30/E)<br>Speed | Gamma | Fog |
|----------------------------------------------------|------------------------|-------|-----|
| dye (g'') alone (.015)                             | 1.3                    | 2.7   | .07 |
| dye (g'') (.015) plus compound 4(3.0)              | 3.5                    | 2.5   | .07 |
| dye (g'') is 3,3'-diethylthiaticarbocyanine iodide |                        |       |     |
|                                                    |                        |       |     |
| Example 41                                         | Red<br>Speed<br>30/E   | Gamma | Fog |
| dye (g'') alone (.010)                             | 3.3                    | 1.4   | .06 |
| dye (g'') (.010) plus Calcofluor White<br>MR (3.0) | 13.7                   | 2.7   | .07 |

In Examples 40 and 41, the amounts are given as g./mol. AgX.

The dicarbocyanine dyes of Formula I above comprise a well known class of optical sensitizing dyes. Methods for making these dyes have been previously described in the prior art. See, for example, U.S. Patent 2,131,865, issued October 4, 1938; U.S. Patent 2,213,238, issued September 3, 1940; U.S. Patent 2,218,450, issued October 15, 1940; U.S. Patent 2,269,234, issued January 6, 1942; and British 562,567, accepted July 6, 1944. The following examples will serve to illustrate these well known methods.

## EXAMPLE 42

## 3,3'-diethyl-5,5'-diphenyloxadidicarbocyanine perchlorate



A mixture of 3.65 g. (2 mol.) of 3-ethyl-2-methyl-5-phenylbenzoxazolium iodide and 1.74 g. (1 mol. plus 100% excess) of 1,3,3-triethoxypropene in 10 ml. of acetic anhydride was heated, with shaking, at the refluxing temperature for about 5 minutes. The cool reaction mixture was stirred with ether, the liquors were decanted and the remaining residue was stirred with hot acetone. After chilling, the solid was collected on a filter and washed with acetone and then water. After one recrystallization from methyl alcohol the dye was converted to the perchlorate by adding a hot aqueous solution of sodium perchlorate to a hot methyl alcoholic solution of the dye. The dye was recrystallized from methyl alcohol. The coppery crystals melted at 234-236° C. with decomposition.

## EXAMPLE 43

## 3-ethyl-3'-β-hydroxyethylthiadicarbocyanine iodide



A mixture of 5.48 g. (1 mol.) of 3-β-hydroxyethyl-2-methylbenzothiazolium bromide, 7.14 g. (1 mol.) of 3-ethyl-2-(4-methoxy-1,3-butadienyl)benzoxazolium iodide and 4.04 g. (1 mol. plus 100% excess) of triethylamine in 50 ml. of absolute ethyl alcohol was stirred at room temperature for 5 minutes. The reaction mixture was filtered and the residue was thoroughly washed with water and then with a little methyl alcohol. The yield of dye was 53% crude and 35% after two recrystallizations from methyl alcohol. The green crystals melted at 250-251° C. with decomposition.

5  
10

5  
10

15  
20  
25  
30

A mixture of 3.49 g. (1 mol.) of 3-ethyl-2-methyl-5-phenylbenzothiazolium p-toluenesulfonate, 4.77 g. (1 mol.) of 3-ethyl-2-(4-methoxy-1,3-butadienyl) - 5 - phenylbenzoxazolium p-toluenesulfonate and 2.02 g. (1 mol. plus 100% excess) of triethylamine in 35 ml. of absolute ethyl alcohol was stirred at room temperature for 5 minutes. After chilling the reaction mixture, it was filtered and the residue was washed with ethyl alcohol. The yield of dye was 100% crude and 74% after two recrystallizations from methyl alcohol. The green needles melted at 221-222° C. with decomposition.

The 3-ethyl-2-(4-methoxy-1,3-butadienyl) - 5 - phenylbenzoxazolium p-toluenesulfonate was prepared as follows. The crude quaternary salt obtained by heating 99.5 g. of 2-methyl-5-phenylbenzoxazole and 100 g. of ethyl p-toluenesulfonate together overnight at 110° C. was dissolved in 500 ml. of acetic acid. Then 132 g. of 1,3,3-triethoxypropene was added and the reaction mixture was heated at the refluxing temperature for 30 minutes. After chilling, with stirring, the intermediate was collected on a filter and washed first with ether and then with acetone. The yield was 74 g.

35

EXAMPLE 44  
3,3'-diethyl-5-phenyloxathiadidicarbocyanine p-toluenesulfonate

40

45  
50  
55

A hot solution of 2.75 g. (1 mol.) of 3-β-hydroxyethyl-2-methylbenzothiazolium bromide in 50 ml. of absolute ethyl alcohol was cooled quickly with stirring to room temperature. Then 4.77 g. (1 mol.) of 3-ethyl-2-(4-methoxy-1,3-butadienyl) - 5 - phenylbenzoxazolium p-toluenesulfonate and 2.02 g. (1 mol. plus 100% excess) of triethylamine were added and the reaction mixture was stirred at room temperature for 10 minutes. The dye was collected on a filter and washed with methyl alcohol. The yield of dye was 77% crude and 49% after two recrystallizations from methyl alcohol. The blue needles with a green reflex melted at 255-256° C. with decomposition.

Listed below are the melting points of dyes used in the above tables, which were prepared in exactly the same manner illustrated in Examples 43-46 above.

| Dye: | Melting point                                                   |
|------|-----------------------------------------------------------------|
| y    | 229-230° C. with decomposition.                                 |
| e'   | 215-216° C. with decomposition.                                 |
| g'   | 236-237° C. with decomposition.                                 |
| i'   | 178-180° C. with decomposition.                                 |
| k'   | 177-178° C. with decomposition.                                 |
| m'   | 220-221° C. with decomposition.                                 |
| o'   | 186-187° C. with decomposition.                                 |
| q'   | 189-191° C. with decomposition and shrinking from about 180° C. |
| s'   | 208-209° C. with decomposition.                                 |
| u'   | 191-195° C. with decomposition and shrinking from about 165° C. |
| c''  | 225-227° C. with decomposition.                                 |
| e''  | 215-216° C. with decomposition.                                 |

75

Dye y' above was prepared according to the method of U.S. Patent 2,269,234 (using intermediate of Example 1 and the benzimidazole quaternary salts of U.S. patent 2,320,439). It melted at 149-155° C. with decomposition.

As noted above the bistriazinylaminostilbene compounds represented by Formula II comprise a well-known class of "optical" bleaching agents, and methods for making them have been fully described in the prior art listed above. This can be illustrated further with reference to the preparation of compound 9 above.

*Step 1.*—Three solutions were prepared as follows:

(a) 260 g. of purified diamino stilbene disulfonic acid in 1 liter of water.



(b) 259 g. of cyanuric chloride in 461 g. of acetone.

(c) 42.6 g. of sodium carbonate in 500 ml. of water.

Solutions (b) and (c) were added to solution (a) at 0° C., with good agitation. Proportions were adjusted to keep the mixture neutral or weakly acid. The reaction was complete when test for amino nitrogen was negative.

At this time the following compound was present:



*Step 2.*—To this reaction product was added separate solutions (d) and (e) as shown below at 0°-10° C.

(d) 206 g. aniline hydrochloride in 275 liters of water.

(e) 100 g. sodium carbonate in 650 ml. of water.

The temperature was allowed to rise to 20-25° C. and agitation continued until no free aniline was present.

At this time then the following compound was present:



*Step 3.*—Added 550 ml. of 15 percent sodium carbonate solution to the reaction mixture from Step 2. Heated to boiling and the acetone distilled off. Heated several hours after the acetone was removed and diluted to 10 liters. Filtered hot.

Saluted out the filtrate and filtered in a filter press without washing. The optical-bleach concentrate was then dried at 70-80° C. and was in the following chemical form:



In a similar manner compound 27 was prepared as above, using concentrated ammonia in place of the ani-

line used in making compound 9. Likewise, compound 28 was made by employing tris (hydroxymethyl) aminomethane in place of aniline (no Step 3 was used). Compound 26 was prepared by a condensation similar to 5 Step 1 wherein compound 9 was prepared, followed by reduction of the resulting tetrachloro compound to give a compound wherein R<sub>2</sub>, R<sub>3</sub>, R<sub>6</sub> and R<sub>7</sub> of Formula II is hydrogen by heating with a zinc-acetic acid reduction mix. Compound 7 was prepared exactly as compound 5 (U.S. 2,582,357) by using 4,4'-diaminostilbene in place of the corresponding stilbene disulfonic acid. Also useful in practicing our invention are compounds represented by Formula II above wherein R<sub>2</sub>, R<sub>3</sub>, R<sub>6</sub> and/or R<sub>7</sub> each represents a heterocyclamino group (e.g., 2-benzothiazylamino, 2-pyridylamino, etc.). Such compounds can be prepared according to the method described in our copending application 540,054, filed on even date herewith.

We have also found that the compounds represented by Formula II above can advantageously be employed in photographic silver halide emulsions, and particularly photographic silver bromide emulsions (negative speed), containing color-forming or coupling compounds of the type described above to prevent or diminish the formation of spontaneous fog which develops upon exposure of the emulsions to high temperatures and humidity. Also, we have found that the compounds of

Formula II have the valuable property of inhibiting the formation of stain which frequently remains after processing of photographic emulsions containing color-forming compounds. The antifoggant and/or antistain action of the compounds of Formula II appears to be unrelated to the supersensitizing effect shown in the above examples. That is, this antifoggant or antistain action appears to take place regardless of the presence of sensitizing dyes



in the photographic emulsions containing the color-forming compounds of the type mentioned above.

The antifoggant and/or antistain action of the compounds of Formula II appears to be particularly outstanding in the presence of color-forming compounds for the magenta or cyan images, i.e., in the presence of magenta or cyan couplers (e.g., such as the magenta and cyan couplers described in U.S. Patent 2,640,776 mentioned above). The antifoggant and antistain action



of the compounds of Formula II is particularly apparent at concentrations of 1 gram of compound per mole of

silver halide or amounts in excess of 1 gram (e.g., from about 1 to 10 grams per mole of silver halide). It has been also found that the compounds of Formula II are particularly useful in combination with color couplers of the water-soluble type (such as the couplers described in U.S. application Serial No. 470,499, filed November 22, 1954, now U.S. Patent No. 2,808,329, granted October 1, 1957). Such couplers when used in the absence of the compounds of Formula II cause sufficiently high fog to make their use difficult in photographic emulsions. However, when using such couplers in the presence of the compounds of Formula II, the fog is reduced to a considerable degree so that such couplers can be employed from a practical standpoint.

The following examples will serve to illustrate the antifoggant and antistaining action of the compounds of Formula II when employed in photographic silver halide emulsions containing color-forming compounds.

#### EXAMPLE 46

A photographic gelatino-silver-chlorobromide emulsion which had been optically sensitized with one of the dyes of the type represented by Formula I above and containing a coupler dispersion of a color-forming compound, such as coupler No. 5 above, was coated on a cellulose acetate film support. Separate batches of the same emulsion were prepared and to these batches were added Calcofluor White in the amounts given below, and these emulsions were also coated on cellulose acetate film supports. Separate portions of the coatings were then exposed both before and after incubation at 120° F. for seven days, 50 percent relative humidity, through a Wratten No. 25 Filter (i.e., a filter which transmits substantially no light shorter than 580 mu.) and a Wratten No. 47 Filter (i.e., a filter which transmits only light between about 355-515 mu.). The coatings were then developed in a color developer, such as that described for Examples 33 to 38 above. Processing was completed in the same manner described for Examples 33 to 38. The speed figures given below for the coatings are for log E values where the log E is measured at a point on the curve where the density is 0.2 above fog. The speed shifts on incubation given in the table were measured as  $\Delta \log E$ . The results which were obtained are as follows:

| Coating | Addenda (g./mole AgX)   | Fresh Stain | 7 Day Incubation |            |       |
|---------|-------------------------|-------------|------------------|------------|-------|
|         |                         |             | Speed Shifts     |            | Stain |
|         |                         |             | Red              | Minus Blue |       |
| (a)     | Control                 | .06         | -.08             | +.12       | .22   |
| (b)     | Calcofluor White (5.0)  | .04         | -.06             | +.04       | .08   |
| (c)     | Calcofluor White (10.0) | .02         | -.10             | ±.00       | .06   |

#### EXAMPLE 47

Separate portions of a negative speed gelatino-silver-bromide emulsion were green sensitized according to the method described in U.S. Patent 2,701,198 or U.S. Patent 2,165,338 (or by a mixture of the dyes shown in these patents). A mixture of couplers, such as couplers Nos. 7 and 8 above, was then added to the emulsions. To certain portions of the emulsions was added a compound of Formula II in the amount given in the table below. The emulsions were then coated on cellulose acetate supports and one group of fresh coatings was exposed on an intensity scale sensitometer through a Wratten No. 58 Filter, i.e., a filter which transmits only light of wavelengths lying between 465 and 620 mu. The remaining coatings as identified in the table, were incubated for

the times shown in the table before exposure. The exposed coatings were then processed in a color developer having the following composition:

|    |                                      |    |      |
|----|--------------------------------------|----|------|
| 5  | Water (70-75° F.)                    | cc | 750  |
|    | Benzyl alcohol                       | cc | 3.8  |
|    | Calgon                               | g  | 2.0  |
|    | Sodium sulfite (anhydrous)           | g  | 2.0  |
|    | Sodium hydroxide (cold 10% solution) | cc | 5.5  |
| 10 | Developer 1                          | g  | 5.0  |
|    | Potassium bromide                    | g  | 1.0  |
|    | Sodium carbonate monohydrate         | g  | 50.0 |
|    | Water to make 1 liter.               |    |      |

<sup>1</sup> 4-amino - N - ethyl - N - (β - methanesulfonamidoethyl)-m-toluidine sesquisulfate monohydrate.

The developed coatings were then fixed and bleached in a potassium dichromate bath in the usual manner. The results given in the table below show the shift in speed ( $\Delta \log E$ , as measured in Example 46) for these coatings. The antifoggant action of the compound of Formula II is self-evident. The 7-day incubation tests were run at 120° F., 50% relative humidity, while the 28-day tests were run at 100° F., 50% relative humidity. The results are as follows:

| Coating | Addenda (g./mole AgX)  | Original Tests |     | Incubation Tests |             |
|---------|------------------------|----------------|-----|------------------|-------------|
|         |                        | Speed          | Fog | Time, Days       | Speed Shift |
| 30      |                        |                |     |                  |             |
| (a)     | Control                |                |     | .17              | .14         |
| (b)     | Calcofluor White (5.0) | -.14           | .10 | 7                | -.10        |
| 35      | (c)                    | Control        |     | .15              | .28         |
| (d)     | Calcofluor White (5.0) | -.15           | .08 | 28               | -.19        |

#### EXAMPLE 48

40 To separate portions of a negative speed gelatino-silver-bromide emulsion of the type normally used in reversal color films was added an optical sensitizing dye of the type shown in U.S. Patent 2,165,338 in the amounts shown in the table below. To each portion of this emulsion was added a dispersion of a color coupler, such as coupler No. 7 above. To certain portions of the emulsion was added the compound of Formula II, in the amounts shown in the table. One group of the coatings was then exposed in an intensity scale sensitometer in exactly the manner described in Example 47 above, while the other group of coatings was incubated for 7 days at 120° F., 50% relative humidity before exposure. The exposed coatings were then reversal processed, first in a conventional black and white developer, such as that shown in 45 Example 32 above and then in a color developer having the following composition:

|    |                                  |       |       |
|----|----------------------------------|-------|-------|
| 60 | Water (70-80° F.)                | liter | 1     |
|    | Benzyl alcohol                   | cc    | 6.0   |
|    | Calgon                           | g     | 2.0   |
|    | Sodium sulfite                   | g     | 5.0   |
|    | Trisodium phosphate              | g     | 40    |
|    | Potassium bromide                | g     | 0.25  |
|    | Potassium iodide (0.1% solution) | cc    | 10.0  |
| 65 | Sodium hydroxide                 | g     | 6.5   |
|    | Developer 1                      | g     | 11.33 |
|    | Ethylenediamine sulfate          | g     | 7.8   |
|    | Citrazinic acid                  | g     | 1.5   |

<sup>1</sup> 4-amino - N - ethyl - N - (β - methanesulfonamidoethyl)-m-toluidine sesquisulfate monohydrate.

The developed coating was then bleached in a conventional potassium dichromate-potassium ferricyanide bleach. The speed and density for each of the coatings was then measured. The speed figures given in the table

below are expressed as  $10/\log E$  where  $\log E$  is measured at a density of 0.3 below D-max. The results follow:

| Coating | Dye (g./mol. AgX) | Calcofluor White (g./mol. AgX) | Fresh Tests |       | 1 Wk. Incubation @ 120° F./50% R.H. |       |        |      |
|---------|-------------------|--------------------------------|-------------|-------|-------------------------------------|-------|--------|------|
|         |                   |                                | D-Max.      | Speed | D-Max.                              | Speed | D-Max. | Loss |
| (a)     | .075              |                                | 1.90        | 5.68  | 1.78                                | 6.67  | -.12   |      |
| (b)     | .150              |                                | 1.86        | 9.17  | 1.63                                | 5.40  | -.23   |      |
| (c)     | .200              |                                | 1.75        | 9.25  | 1.56                                | 8.4   | -.19   |      |
| (d)     | .075              | 10.0                           | 1.98        | 7.75  | 1.97                                | 7.69  | -.01   |      |
| (e)     | .150              | 10.0                           | 2.02        | 8.55  | 2.02                                | 9.28  | +.00   |      |
| (f)     | .200              | 10.0                           | 2.00        | 8.70  | 2.00                                | 8.33  | +.04   |      |

#### EXAMPLE 49

To separate portions of a gelatino-silver-bromiodide emulsion which had been green sensitized with a dye of the type described in U.S. Patent 2,241,237 or 2,165,338 (or a mixture of such dyes) were added coupling com-

100° F., 50% relative humidity. The emulsions were then exposed exactly as described in Example 46 above,

and processed as described in Example 46. The dicarboxylic dye used in this example was of the type described in U.S. Patent 2,213,238, while the merocyanine 20 dye was of the type described in U.S. Patent 2,282,116. The results obtained were as follows:

| Coating | Dye          | Addenda (g./mol. AgX) | Fresh Tests, Log E Shifts |            | Incubation Tests |                |            |
|---------|--------------|-----------------------|---------------------------|------------|------------------|----------------|------------|
|         |              |                       | Red                       | Minus Blue | Time, Days       | Δ Log E Shifts |            |
|         |              |                       |                           |            |                  | Red            | Minus Blue |
| (a)     | none         |                       |                           |            | 7                | +.30           | +.04       |
| (b)     | none         |                       |                           |            | 7                | +.24           | +.02       |
| (c)     | none         |                       |                           |            | 7                | +.22           | +.00       |
| (d)     | dicarboxylic |                       |                           |            | 7                | +.08           | +.04       |
| (e)     | do           |                       |                           |            | 7                | +.06           | +.00       |
| (f)     | do           |                       |                           |            | 7                | +.02           | +.04       |
| (g)     | merocyanine  |                       |                           |            | 28               | +.02           | +.08       |
| (h)     | do           |                       |                           |            | 28               | +.04           | +.04       |
| (i)     | do           |                       |                           |            | 28               | +.02           | +.00       |

pounds of the type indicated in the following table. To certain portions of the emulsions was added a compound of Formula II in the amounts indicated in the table. The emulsions were then coated on cellulose acetate supports and exposed in an intensity scale sensitometer as described in Example 47 above. The exposed emulsions were then processed in exactly the same manner shown in Example 47. The results obtained are illustrated in the following table:

| Coating | Couplers | Calcofluor White (g./mol. AgX) | Speed Shift Δ Log E | Fog |
|---------|----------|--------------------------------|---------------------|-----|
| (a)     | 7+8      | none                           |                     | .26 |
| (b)     | 7+14     | none                           | -.48                | .65 |
| (c)     | 7+14     | 5                              | -.14                | .55 |
| (d)     | 7+14     | 1.0                            | -.16                | .44 |
| (e)     | 7+14     | 2.0                            | -.10                | .30 |
| (f)     | 7+14     | 5.0                            | -.14                | .24 |

14=1-phenyl-3-(2-carboxybenzamido)-4-(p-dodecyloxyphenylazo)-5-pyrazolone.

#### EXAMPLE 50

To separate portions of a positive speed gelatino-silver-chlorobromide emulsion was added a color coupler, such as coupler No. 5 above. To some of these portions was added an optical sensitizing dye, as indicated in the table below, as well as a compound of Formula II. The emulsions were then coated on a conventional cellulose acetate support. Some of the emulsions were exposed immediately after coating and drying, while some of the emulsions were exposed only after incubation, as set forth in the table. The coatings incubated for 7 days were exposed to a temperature of 120° F., 50% relative humidity, while the coatings incubated for 28 days were held at

45 The accompanying drawings illustrates the supersensitizing effect obtained with three of our new combinations in gelatino-silver-bromiodide emulsions. Each figure in the drawing is a diagrammatic reproduction of one or two (Fig. 1) spectrograms. The sensitivity of the emulsion containing only the dicarboxylic dye represented by Formula I is represented by the broken line in Fig. 1, while the sensitivity of the same emulsion containing both a dicarboxylic dye of Formula I and the triazine compound of Formula II is represented by the 50 solid curve. No curve for the emulsion containing the triazine compound of Formula II alone is given, since it has been found that these compounds alone generally have little or no measurable sensitizing effect on the emulsions. The same sensitizing dye was employed in the 55 coatings of Fig. 2 and Fig. 3 as was used in Fig. 1, hence curve A of Fig. 1 is not reproduced in Figs. 2 and 3 since it would merely be identical thereto.

In Fig. 1, curve A represents the sensitivity of an ordinary gelatino-silver-bromiodide emulsion containing 3,3'-diethyloxathiadicarboxylic iodide, while curve B represents the sensitivity of the same emulsion sensitized with 3,3'-diethyloxathiadicarboxylic iodide and 4,4'-bis(4,6-dianilino-s-triazin-2-ylamino)stilbene-2,2'-disulfonic acid.

In Fig. 2, curve C represents the sensitivity of an ordinary gelatino-silver-bromiodide emulsion sensitized with 3,3'-diethyloxathiadicarboxylic iodide and 4,4'-bis(4-phenoxy-6-β-hydroxyethylamino-s-triazin-2-ylamino)stilbene-2,2'-disulfonic acid. The sensitometric measurements for the coatings of Figs. 1, 2 and 3 are given in Examples 2, 4 and 5 of Table I above.

By bis(s-triazin-2-ylamino)stilbene compound, we mean a compound of the following structure:



wherein R<sub>4</sub> and R<sub>5</sub> each have the values given above, and D and D<sub>1</sub> each represents a s-triazin-2-yl nucleus.

The disulfonic acids of Formula II are generally employed in neutral aqueous solution as mentioned above, i.e., the free acids are at least partially neutralized with sodium hydroxide, potassium hydroxide, sodium carbonate, ammonia, triethylamine, etc. before use in the emulsions. The corresponding disulfonic acid salts result. It is thus possible to adjust the pH of these aqueous solutions so that they are about the same as the pH of the emulsions.

What we claim as our invention and desire secured by Letters Patent of the United States is:

1. A photographic silver halide emulsion sensitized with a supersensitizing combination of at least one dicarbocyanine dye selected from the class represented by the following general formula:



wherein R and R<sub>1</sub> each represents an alkyl group containing not more than four carbon atoms, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the naphthothiazole series, those of the benzoxazole series, those of the naphthoxazole series, those of the benzoselenazole series, and those of the naphthoselenazole series, and at least one bis(s-triazin-2-ylamino)-stilbene selected from the class represented by the following general formula:



wherein R<sub>2</sub>, R<sub>3</sub>, R<sub>6</sub> and R<sub>7</sub> each represents a member selected from the group consisting of a hydrogen atom, a hydroxyl group, an aryloxy group, an alkoxy group, a halogen atom, a heterocyclic radical an alkylthio group, an arylthio group, and an amino group and R<sub>4</sub> and R<sub>5</sub> each represents a member selected from the group consisting of a hydrogen atom and a sulfo group.

2. A photographic silver halide emulsion sensitized with a supersensitizing combination of at least one dicarbocyanine dye selected from the class represented by the following general formula:



wherein R and R<sub>1</sub> each represents an alkyl group containing not more than four carbon atoms, n represents a positive integer of from 1 to 2, X represents an acid radical, Z represents the non-metallic atoms necessary to complete a heterocyclic nucleus selected from the group consisting of those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the naphthothiazole series, those of the benzoxazole series, those of the naphthoxazole series, those of the benzoselenazole series, and those of the naphthoselenazole series, and at least one bis(s-triazin-2-ylamino)-stilbene selected from the class represented by the following general formula:

group consisting of those of the benzothiazole series, those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the naphthothiazole series, those of the benzoxazole series, those of the naphthoxazole series, those of the benzoselenazole series, those of the naphthoselenazole series, and those of the 2-quinoline series, those of the 4-quinoline series, those of the benzimidazole series, and those of the 5,6-benzoquinoline series, and at least one bis(s-triazin-2-ylamino)-stilbene selected from the class represented by the following general formula:



20 wherein D and D<sub>1</sub> each represents a s-triazin-2-yl nucleus.

3. A photographic gelatino-silver-bromide emulsion sensitized with a supersensitizing combination of at least one dicarbocyanine dye selected from the class represented by the following general formula:



30 wherein R and R<sub>1</sub> each represents an alkyl group containing from 1 to 2 carbon atoms, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the naphthothiazole series, those of the benzoxazole series, those of the naphthoxazole series, those of the benzoselenazole series, and those of the naphthoselenazole series, and at least one bis(s-triazin-2-ylamino)-stilbene selected from the class represented by the following general formula:



wherein D and D<sub>1</sub> each represents a s-triazin-2-yl nucleus.

4. A photographic gelatino-silver-chlorobromide emulsion sensitized with a supersensitizing combination of at least one dicarbocyanine dye selected from the class represented by the following general formula:



50 wherein R and R<sub>1</sub> each represent an alkyl group containing from 1 to 2 carbon atoms, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the naphthothiazole series, those of the benzoxazole series, those of the naphthoxazole series, those of the benzoselenazole series, and those of the naphthoselenazole series, and at least one bis(s-triazin-2-ylamino)-stilbene selected from the class represented by the following general formula:

70 wherein R and R<sub>1</sub> each represents an alkyl group containing not more than four carbon atoms, n represents a positive integer of from 1 to 2, X represents an acid radical, Z represents the non-metallic atoms necessary to complete a heterocyclic nucleus selected from the group consisting of those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the naphthothiazole series, those of the benzoxazole series, those of the naphthoxazole series, those of the benzoselenazole series, and those of the naphthoselenazole series, and at least one bis(s-triazin-2-ylamino)-stilbene selected from the class represented by the following general formula:

75 wherein R and R<sub>1</sub> each represents an alkyl group containing not more than four carbon atoms, n represents a positive integer of from 1 to 2, X represents an acid radical, Z represents the non-metallic atoms necessary to complete a heterocyclic nucleus selected from the group consisting of those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the naphthothiazole series, those of the benzoxazole series, those of the naphthoxazole series, those of the benzoselenazole series, and those of the naphthoselenazole series, and at least one bis(s-triazin-2-ylamino)-stilbene selected from the class represented by the following general formula:



stillbene compound selected from the class represented by the following general formula:



wherein R<sub>2</sub>, R<sub>3</sub>, R<sub>6</sub> and R<sub>7</sub> each represents a member selected from the group consisting of a hydrogen atom, a hydroxyl group, an aryloxyl group, an alkoxyl group, a halogen atom, a heterocyclic radical, an alkylthio group, an arylthio group and an amino group, and R<sub>4</sub> and R<sub>5</sub> each represents a member selected from the group consisting of a hydrogen atom and a sulfo group, said bis(s-triazin-2-ylamino)stilbene compound being incapable of coupling with the oxidation products of a primary aromatic amine developing agent to provide a dye image.

References Cited in the file of this patent

UNITED STATES PATENTS

|           |          |                |
|-----------|----------|----------------|
| 2,271,623 | Carroll  | Feb. 3, 1942   |
| 2,367,551 | Yule     | Jan. 16, 1945  |
| 2,397,867 | Jennings | Apr. 2, 1946   |
| 2,418,747 | Bailey   | Apr. 8, 1947   |
| 2,476,536 | Dersch   | July 19, 1949  |
| 2,701,198 | Carroll  | Feb. 1, 1955   |
| 2,718,466 | Wolfson  | Sept. 20, 1955 |

FOREIGN PATENTS

|         |               |               |
|---------|---------------|---------------|
| 675,656 | Great Britain | July 16, 1952 |
| 878,823 | France        | Nov. 2, 1942  |

OTHER REFERENCES

Mees: "The Theory of the Photographic Process," MacMillan Co., N.Y., 1954, page 365.

UNITED STATES PATENT OFFICE  
CERTIFICATE OF CORRECTION

Patent No. 2,945,762

July 19, 1960

Burt H. Carroll et al.

It is hereby certified that error appears in the printed specification of the above numbered patent requiring correction and that the said Letters Patent should read as corrected below.

Column 3, line 66, for "stilzene" read -- stilbene --; column 5, line 28, after "dye" insert -- to --; column 10, line 10, after "0.3" insert -- above --; column 11, line 4, for "follows" read -- follow --; column 13, lines 46 to 55, Step 2, the left-hand portion of the formula should appear as shown below instead of as in the patent:



column 18, line 40, for "drawings" read -- drawing --; line 53, for "measureable" read -- measurable --; column 20, line 40, after "complete" insert -- a --; line 62, for "represent" read -- represents --; column 21, line 47, for "af" read -- of --; column 22, line 39, for "lyamino)" read -- ylamino) --.

(SEAL)

Signed and sealed this 18th day of April 1961.

Attest:

ERNEST W. SWIDER  
Attesting Officer

DAVID L. LADD  
Commissioner of Patents